

# United States Patent [19]

Tan et al.

[11] 3,820,988

[45] June 28, 1974

- [54] **METHOD OF SENSITIZING ZINC TELLURIDE**
- [75] Inventors: **Yen T. Tan; Rajinder P. Khosla; John R. Fischer; Deepak K. Ranadive**, all of Rochester, N.Y.
- [73] Assignee: **Eastman Kodak Company**, Rochester, N.Y.
- [22] Filed: **Mar. 13, 1972**
- [21] Appl. No.: **234,382**
- [52] U.S. Cl. .... **96/1.5**, 250/501, 423/508, 423/509
- [51] Int. Cl. .... **G03g 5/02**, G03g 5/04
- [58] Field of Search..... 252/501; 96/1 R, 1 PC, 96/1.5; 423/508, 509

[56] **References Cited**

UNITED STATES PATENTS

- 2,994,621 8/1961 Hugle et al. .... 252/501 X

|           |         |                      |           |
|-----------|---------|----------------------|-----------|
| 3,104,229 | 8/1963  | Koelmans et al. .... | 252/501   |
| 3,174,823 | 3/1965  | Kopelman ....        | 423/509   |
| 3,188,594 | 6/1965  | Koller et al. ....   | 252/501 X |
| 3,462,323 | 8/1969  | Groves ....          | 423/509 X |
| 3,551,763 | 12/1970 | Hakki ....           | 423/508 X |

**OTHER PUBLICATIONS**

Bube and Lind, "CdS-Type Photoconductivity in ZnTe Crystals," Phys. Rev. 105, pp. 1711-1712 (1957).

Makarenko et al., "Some Features of the Photoconducting of ZnTe Crystals Under Combined Excitation Conditions," Soviet Phys. Semiconductors, 4, p. 847-848, (1970).

*Primary Examiner*—Roland E. Martin, Jr.  
*Attorney, Agent, or Firm*—Dennis M. DeLeo

[57] **ABSTRACT**

Zinc telluride can be sensitized by annealing in the presence of vapors of both zinc metal and a Group IIIA metal dopant. The sensitized zinc telluride exhibits photoconductivity.

**5 Claims, No Drawings**

## METHOD OF SENSITIZING ZINC TELLURIDE

## FIELD OF INVENTION

This invention relates to semiconductors and to methods for preparation thereof. In particular, this invention relates to means for preparing p-type semiconductors which exhibit photoconductivity.

## DESCRIPTION OF PRIOR ART

Zinc telluride is a well known compound. Pure zinc telluride is relatively electrically conductive and is not particularly photoconductive. Various attempts have previously been made to alter zinc telluride. For example, Bube and Lind in Phys. Rev. 105, 1711, (1957), first observed photoconductivity in zinc telluride crystals which are doped with indium and aluminum. Further work done by Makaranko and Rybalka reported in Soviet Physics, Semiconductors, 4, 847, (1970) involved infrared quenching in zinc telluride which contained iodine, indium or gallium impurities. Although some photoresponse was noticed in these works, the observed photocurrent was relatively small. Bube and Lind, for instance, reported a current of only 40 microamps with an applied voltage of 100 volts and an intensity of 1.5 mw/cm<sup>2</sup>. Although this prior work is interesting, there still exists a need for techniques to prepare zinc telluride crystals having relatively high photoconductivity.

## SUMMARY OF THE INVENTION

We have found that essentially pure zinc telluride can be rendered photoconductive by an annealing technique. This process results in a p-type semiconductor having useful photoconductive properties. The resultant p-type materials are useful in electrophotography, in semiconductor junction devices, in photoconductive cells and the like. In addition, the present process provides a means for varying the temperature for peak photosensitivity of the compound by varying the annealing time.

## DESCRIPTION OF THE PREFERRED EMBODIMENTS

The objects of the present invention are accomplished by a process of annealing zinc telluride in the presence of vapors of zinc and vapors of a dopant followed by cooling. The dopant used in this invention is a Group IIIA metal such as gallium and indium, etc.

In accordance with this invention, the zinc telluride to be treated is placed in a sealed container and annealed at elevated temperatures in the presence of vapors of both zinc and a Group IIIA metal. The annealing can be carried out at temperatures between about 600°C and the melting point of the zinc telluride. The material can be treated at temperatures below about 600°C, but the time required to produce useful results (e.g., to reduce the hole concentration sufficiently) becomes excessive. At temperatures above about 950°C, the material begins to evaporate and special precautions must be taken to prevent condensation on cooler portions of the container. From the standpoint of efficiency, the preferred annealing temperature range is about 750° to about 900°C.

The exact mechanism of the present process is not fully understood at this time. However, it appears to be a combined effect of a reduction of hole concentration

by the presence of zinc and the addition of electron donors which increase the so-called compensation ratio. As mentioned above, pure zinc telluride has a relatively high conductivity. This is believed to be the result of native acceptors near the valence band. These native acceptors, which are theorized as being zinc vacancies, allow hole migration in the valence band giving rise to conductivity. In order to reduce this conductivity, we anneal in the presence of zinc and a Group IIIA metal.

10 The presence of the zinc vapor during the annealing process tends to reduce the concentration of native acceptors which aids in the reduction of conductivity. In addition, we introduce an impurity (that is, a Group IIIA metal dopant) within the band gap of the zinc telluride crystal. The introduction of this dopant into the band gap results in compensation of the native acceptor by the ionization of the donor dopant.

15 After suitable annealing, the zinc telluride is quenched to rapidly cool the annealed compound to about room temperature. The material is quenched while the zinc telluride is maintained in the sealed container with the zinc vapor and Group IIIA metal vapor.

This quenching is done in order to maintain the high temperature defect structure of the treated crystal. A typical time for annealing prior to quenching would be a minimum of about 10 hours. The material must be annealed for a period of time sufficiently long so that the zinc and Group IIIA dopant will diffuse beneath the surface of the zinc telluride crystal. For practical purposes, 20 hours is a preferred minimum to insure sufficient diffusion beyond the surface. The material can be annealed for as long as about 150 hours. Further annealing beyond this does not give rise to any significant change in properties.

25 By varying the annealing time, one can vary the temperature for peak photosensitivity. This allows one to essentially obtain a material having a peak photosensitivity at a different temperature.

30 The starting zinc telluride crystal should be pure material. It may be off-stoichiometric, but should contain no more than about 0.3 mole percent excess of tellurium. If a greater excess than this is present, the time of annealing is changed significantly and difficulties arise in achieving a product useful as a photoconductor or the like. It appears that the presence of a large excess of tellurium essentially negates the effect of the presence of the zinc vapors during annealing and poor results are thus obtained.

35 Zinc telluride crystals useful for treatment by the present invention can be prepared by standard techniques known in the art. The zinc telluride crystals can conveniently be prepared by the procedures of J. Steininger and R. E. England as described in "Growth of Single Crystals of ZnTe and ZnTe<sub>1-x</sub>Se<sub>x</sub> by Temperature Gradient Solution Zoning," *Transactions of the Metallurgical Society of AIME*, Volume 242, page 444 (1968). Evaporated layers of zinc telluride can also be treated by the process of this invention.

40 The starting zinc telluride crystal should be pure material. It may be off-stoichiometric, but should contain no more than about 0.3 mole percent excess of tellurium. If a greater excess than this is present, the time of annealing is changed significantly and difficulties arise in achieving a product useful as a photoconductor or the like. It appears that the presence of a large excess of tellurium essentially negates the effect of the presence of the zinc vapors during annealing and poor results are thus obtained.

45 Zinc telluride crystals useful for treatment by the present invention can be prepared by standard techniques known in the art. The zinc telluride crystals can conveniently be prepared by the procedures of J. Steininger and R. E. England as described in "Growth of Single Crystals of ZnTe and ZnTe<sub>1-x</sub>Se<sub>x</sub> by Temperature Gradient Solution Zoning," *Transactions of the Metallurgical Society of AIME*, Volume 242, page 444 (1968). Evaporated layers of zinc telluride can also be treated by the process of this invention.

50 The starting zinc telluride crystal should be pure material. It may be off-stoichiometric, but should contain no more than about 0.3 mole percent excess of tellurium. If a greater excess than this is present, the time of annealing is changed significantly and difficulties arise in achieving a product useful as a photoconductor or the like. It appears that the presence of a large excess of tellurium essentially negates the effect of the presence of the zinc vapors during annealing and poor results are thus obtained.

55 Zinc telluride crystals useful for treatment by the present invention can be prepared by standard techniques known in the art. The zinc telluride crystals can conveniently be prepared by the procedures of J. Steininger and R. E. England as described in "Growth of Single Crystals of ZnTe and ZnTe<sub>1-x</sub>Se<sub>x</sub> by Temperature Gradient Solution Zoning," *Transactions of the Metallurgical Society of AIME*, Volume 242, page 444 (1968). Evaporated layers of zinc telluride can also be treated by the process of this invention.

60 The following embodiments are included for a further understanding of the invention.

Embodiment 1  
Crystals of zinc telluride are grown from 99.9999 percent pure zinc and tellurium by an off-stoichiometry Bridgman method as described by Steininger and England (supra). A charge of the pure zinc and tellurium metals, with about 10 percent excess of tellurium, is placed in a vacuum sealed quartz ampoule. The ampoule is placed in a two-zone furnace and

driven through a temperature gradient of 25°C/in. The crystals thus formed contain about 0.12 percent excess tellurium. The bulk crystals are cut into Hall spiders about 1mm thick and weighing about 0.1 to about 0.3 grams. The resultant Hall spiders are placed in a quartz vacuum ampoule about 5 to 10 cc. in size with about 0.2 grams of zinc metal of the purity used to make the original crystal and about 0.1 gram of similarly pure gallium metal. The ampoule is evacuated to about  $1 \times 10^{-5}$  torr and sealed. The ampoule is then annealed at about 835°C for about 39 hours and quickly quenched to room temperature in an oil bath. The annealed sample is then removed and etched in concentrated solution of hot sodium hydroxide. Lithium contacts are applied by placing a small drop of  $10^{-4}$  molar LiNO<sub>3</sub> solution on the contact area and then heating the sample in a flowing hydrogen atmosphere at about 350°C for a minute. This technique is described by Aven and Garwacki in J. Electrochem. Soc., 14, 1063 (1967). Electroless gold from an HAuCl<sub>4</sub> solution is deposited on the lithium contacts. The resultant lithium-gold electrodes give good, low resistance ohmic contacts over a range of temperatures. The dark resistance of the sample is measured and found to be greater than  $10^7$  ohms. The photoresponse is measured by determining the specific sensitivity S of the sample. Specific sensitivity, as described by R. H. Bube, RCA Eng., 5, 28 (1960), is defined as  $S = \Delta i l^2 / VP$  where  $\Delta i$  is the change in photocurrent, l is the distance between electrodes, V is the applied voltage and P is the light absorbed in watts. The specific sensitivity is independent of the applied field and the intensity of the illumination if both vary linearly with photocurrent. The applied field is varied between 2 to 20 v/cm. The specific sensitivity is calculated for samples illuminated with a tungsten source and a monochrometer at 560 nm. The intensity of illumination is about 1 mw/cm<sup>2</sup>. The result of these measurements indicate the specific sensitivity at room temperature to be 0.02. The peak specific sensitivity at 200°K is 0.7, which compares with the peak specific sensitivity of 0.1 to 2.0 obtained with highly sensitized cadmium sulfide. A bulk sensitivity may be calculated for the non-current-carrying electrodes of the Hall spider in order to exclude contact resistance. The bulk sensitivity  $S_b$  is defined by the following equation:  $S_b = \Delta\sigma(Al)^2/p$  where  $\Delta\sigma$  is the bulk photoconductivity and A is the cross-sectional area. The bulk sensitivity of the sample is 1.6 at about 200°K and 560 nm.

#### Embodiment 2

Embodiment 1 is repeated with the exception that the sample is annealed for 64 hours and the peak specific sensitivity is 0.16 and the bulk sensitivity is 2.9.

#### Embodiment 3

Embodiment 1 is repeated except that the sample is annealed for 99 hours with the resultant peak bulk sensitivity of 2.2 at room temperature and about 560 nm. The dark resistance is  $10^{10}$  ohms.

#### Control No. 1

Embodiment 1 is repeated with the exception that the ampoule contains only zinc telluride and gallium metal. The ampoule is annealed for 64 hours and quenched as previously. There is practically no photoconductivity at room temperature of the resultant sample and the peak specific sensitivity is  $10^{-6}$  at about 143°K and about 560 nm.

#### Control No. 2

Embodiment 1 is repeated once more except that the ampoule contains only zinc telluride and zinc metal with annealing for about 50 hours. The specific sensitivity at 90°K is about  $10^{-4}$  for the resultant material and the dark resistance is about 300 ohms.

#### Control No. 3

Embodiment 1 is repeated except that the sample is not subjected to annealing. There is no noticeable photosensitivity and the ratio of light to dark conductivities (signal to noise ratio) is less than 1.01. The dark resistance is about 150 ohms.

#### Embodiment 4

Embodiment 1 is repeated with the exception that the ampoule contains zinc telluride, zinc metal and indium metal and is annealed for about 63 hours at 850°C. The resultant sample shows a peak specific sensitivity of 0.08 and a bulk sensitivity of 2.3 at 165°K and 560 nm.

#### Control No. 4

Embodiment 4 is repeated with the exception that the ampoule contains zinc telluride and indium metal only and is annealed for 62 hours at 835°C. The resultant sample shows practically no photosensitivity at room temperature and a peak specific sensitivity of about  $10^{-3}$  at 154°K and 560 nm.

#### Embodiment 5

The annealed zinc telluride formed by the procedure of Embodiment 1 is ground into a powder and combined with an electrically insulating polymeric binder and coated onto a conductive support. The resultant electrophotographic element is then charged under a corona charger and subjected to illumination. The charge applied to the element is dissipated in the areas of exposure in a manner proportional to the amount of illumination received.

The invention has been described in detail with particular reference to certain preferred embodiments thereof, but it will be understood that variations and modifications can be effected within the spirit and scope of the invention.

#### We claim:

1. A method of preparing photoconductive zinc telluride consisting essentially of the steps of:

1. annealing zinc telluride crystals, having no greater than about 0.3 mole percent excess tellurium, said annealing occurring

a. at a temperature in the range of about 600°C to the melting point of said zinc telluride,

b. for at least about 10 hours and

c. in the presence of vapors of zinc and a Group IIIa metal dopant, wherein said vapors of zinc and Group IIIa metal dopant are present at the saturation vapor pressure for the temperature of said annealing; and

2. quenching to cool said annealed zinc telluride.

2. The method as described in claim 1 wherein said annealing occurs at a temperature in the range of about 750°C to about 900°C.

3. The process as described in claim 1 wherein said dopant is selected from the group consisting of gallium and indium.

4. A photoconductive zinc telluride compound consisting essentially of zinc telluride which has been annealed in the presence of a gaseous Group IIIA metal dopant by the process of claim 1.

5. The method as described in claim 1 wherein said resultant annealed zinc telluride has a peak specific sensitivity of greater than  $10^{-3}$ .